

## UNITED STATES PATENT OFFICE

2,105,274

PROCESS OF PREVENTING YELLOW STAIN  
IN PHOTOGRAPHIC PREPARATIONS AND  
REGULATION OF THE HALOGEN CON-  
TENT THEREOFAlbert Steigmann, Luxembourg-Ville, Luxembourg,  
assignor to Felix Sager & Dr. Gossler Gesell-  
schaft mit beschränkter Haftung, Heidelberg,  
Germany, a firm of GermanyNo Drawing. Application November 7, 1936, Se-  
rial No. 109,792. In Germany December 13,  
1935

14 Claims. (Cl. 95—88)

This invention relates to a product and process of preventing yellow stain in photographic preparations and to the regulation of the halogen content thereof.

5 Thallium salts have been used for the removal of undesirable halogen ions such as excess bromine or iodine ions from developers or fixing baths and other photographic solutions. These thallium salts, such as thallous nitrate or acetate 10 form difficulty soluble halides. However, the use of thallium salts has a tendency to form fog in photographic emulsions which is undesirable.

I have discovered that iodonium compounds have all the good properties of the thallium salts 15 when used in photographic solutions and they also act to prevent fog and particularly yellow stain, while at the same time, they do not interfere in the least with sensitivity and gradation. Furthermore, the use of iodonium com- 20 pounds, during developing brings about a precipitation of silver in the deepest blacks that are non-bronzing and which are free from reflection.

I have found that the use of suitable iodonium salts such as diphenyl iodonium nitrate or acetate in photographic preparations makes it possible 25 to keep the content of halogen ions at a constant value corresponding to the solubility of the iodonium halides in the particular solution. In this manner, an excess of halogen ions in 30 the production of photographic emulsions is prevented from the start, which is of considerable importance in the preparation of, for example, silver iodide emulsions. The influence upon the formation of the grain is also important. If iodonium salts in slight quantities are added after mixing, ripening and subsequent 35 ripening can be carried out at a constant low content of halogen ions. Also, when iodonium compounds are added after ripening, or to the 40 wash water, washing out can be effected at a constant low content of halogen ions, whereby considerable inequalities in washing out the halogen ions in the outer layers can be avoided.

The addition of these iodonium compounds 45 to a developer also prevents the troublesome concentration of potassium bromide or iodide. Similarly such addition to the fixing bath prevents concentration of iodine ions which delays fixing. Furthermore the addition of iodonium com- 50 pounds to fixing baths which have been desilverized and used serves to regenerate the baths so that they may be used again.

In addition to the aforementioned desirable properties being secured in emulsions and devel- 55 opers by the use of iodonium compounds therein,

these compounds have a marked anti-fog effect when added thereto. This anti-fog effect is present even when the iodonium compounds are added to other than the emulsion, as for example to the protective layer, the backing or even to the 5 paper support for the emulsion.

Furthermore I have found that all of the aforementioned advantages can be secured by the addition of other compounds which, due to decomposition and/or mutual reaction of the 10 decomposition products produce iodonium compounds. As an example of such other compound, I find that iodosobenzene, in the cold, disintegrates into iodoxybenzene and iodobenzene and these two products react to form the diphenyl 15 iodonium compound in the developer.

The following are two examples of practicing my invention:

## Example 1

To a silver chloride emulsion, after mixing 20 and prior to ripening add 0.15 to 0.20 grams of diphenyl iodonium nitrate per litre of emulsion. An emulsion thus prepared will not show the least tendency to form yellow stain even during 25 prolonged development.

## Example 2

To a regular metol-hydroquinone developer such as used for papers, add 0.10 to 0.15 grams 30 of diphenyl iodonium acetate to each litre of developer solution which is ready for use. Papers tending to form yellow stain can be satisfactorily developed in this solution even if submerged therein for a prolonged period. Also the formation of bromine and iodine ions which interfere with development is prevented, as these 35 ions precipitate as difficulty soluble diphenyl iodonium bromide or iodide. If necessary, the amount of iodonium compound can be increased according to the quantity of potassium bromide 40 and iodide formed.

I claim:

1. The method of preventing yellow stain and regulating the halogen ions in light sensitive 45 silver halide emulsions, which consists in treating said emulsions with a solution containing a soluble iodonium compound.
2. The method of preventing yellow stain and regulating the halogen ions in light sensitive silver halide emulsions which consists in adding a 50 soluble iodonium compound thereto.
3. The method of preventing yellow stain and regulating the halogen ions in light sensitive silver halide emulsions which consists in adding thereto diphenyl-iodonium nitrate. 55

4. The method of preventing yellow stain and regulating the halogen ions in light sensitive silver halide emulsions which consists in adding thereto diphenyl-iodonium acetate. 5
5. The method of preventing yellow stain and regulating the halogen ions in developers which consists in developing an exposed light sensitive silver halide layer in a solution containing a developing agent and a soluble iodonium compound. 10
6. The method of preventing yellow stain and regulating the halogen ions in developers which consists in adding iodosobenzene to a solution containing a developing agent capable of developing silver halide, said iodosobenzene disintegrating in the cold into iodoxybenzene and iodo-benzene, these two products reacting to form a diphenyl-iodonium compound, and developing an exposed light sensitive silver halide layer in 15 said solution. 20
7. The method of preventing yellow stain and regulating the halogen ions in developers which consists in developing an exposed light sensitive silver halide layer in a solution containing a developing agent and diphenyl-iodonium nitrate. 25
8. The method of preventing yellow stain and regulating the halogen ions in developers which consists in developing an exposed light sensitive silver halide layer in a solution containing a developing agent and diphenyl-iodonium acetate. 30
9. The method of preventing yellow stain and regulating the halogen ions in fixing baths which consists in treating an exposed and developed photographic element in a solution containing a silver halide solvent and a soluble iodonium compound. 10
10. The method of preventing yellow stain and regulating the halogen ions in fixing baths which consists in treating an exposed and developed photographic element in a solution containing a silver halide solvent and diphenyl-iodonium ni- 15
11. The method of preventing yellow stain and regulating the halogen ions in fixing baths which consists in treating an exposed and developed photographic element in a solution containing a silver halide solvent and diphenyl-iodonium acetate. 15
12. A photographic light sensitive element comprising silver halide emulsion, and a soluble iodonium compound therein for preventing yel- 20
13. A photographic developer comprising a developing agent capable of developing a silver halide image, and a soluble iodonium compound therein for preventing yellow stain and regulat- 25
14. A photographic fixing bath comprising a silver halide solvent, and a soluble iodonium compound therein for preventing yellow stain and regulating the halogen ions. 30

ALBERT STEIGMANN.